

March 25, 1924.

1,487,933

C. E. GOODWIN

RAZOR STROP

Filed April 14, 1920

Fig. 1

Fig. 2

Fig. 5



Fig. 3

Fig. 4



Witness  
G. G. Holly

Inventor  
Charles E. Goodwin  
by  
James P. Townsend  
his atty.

## UNITED STATES PATENT OFFICE.

CHARLES E. GOODWIN, OF SANTA ANA, CALIFORNIA, ASSIGNOR TO W. E. OWNBY, OF WINTHROP, IOWA.

## RAZOR STROP.

Application filed April 14, 1920. Serial No. 373,985.

*To all whom it may concern:*

Be it known that I, CHARLES E. GOODWIN, a citizen of the United States, residing at Santa Ana, in the county of Orange and State of California, have invented and discovered a new and useful Razor Strop, of which the following is a specification.

An object of this invention is to provide a novel razor strop by means of which a superior cutting edge can be put onto a razor which is at the beginning of the stropping so dull as to require honing. That is to say, an object of this invention is to provide for the use of barbers, a razor strop which will practically supersede the hone.

A broadly new, pioneer and basic feature of this novel strop is that the stropping surface is provided with a wavy, smooth finish as distinguished from either a flat finish or a corrugated finish, and I have discovered that such finish can be imposed upon good strop leather by bending a strap of such leather suitable for a strop, over a form having a convex rounded surface while the leather is wet, and then working the convex surface of the bent strap with a piece of pumice stone until the surface worked upon is smooth, and hard and conformed to the curvature of the form; and then bringing the strap to a practically straight form whereby the worked surface is given a condensed finely waved undulating structure. A smooth wavy surface is preferably thus made upon the flesh side of the strap.

The purpose of supporting the bent leather on a convex rounded surface and working the convex surface of the bent strap while wet with a piece of pumice stone is to uniformly stretch the worked surface and compress the supported surface so that when the strap is again straightened after the surface has become smooth and hard the required condensed finely waved undulating structure will be prominent in the strap.

Other objects, advantages and features of invention may appear from the accompanying drawing, the subjoined detail description and the appended claims.

The following is a description of the invention and the method of making the same, reference being had to the accompanying drawing.

Figure 1 is a view of the strop looking at the treated surface.

Fig. 2 is an edge view of the strop, the 55 treated surface being at the left side.

Fig. 3 is a greatly magnified fragmental section of the strop shown in Figs. 1 and 2, the treated surface being on the left.

Fig. 4 is a fragmental magnified view of 60 the treated face of the strop shown in Figs. 1, 2 and 3.

Fig. 5 is a fragmental view of a strap as the same may be held in condition for treatment to produce the wavy surface strop. 65

In the several views, 1 indicates the strop, 2 indicates the condensed, smooth, wavy, flesh side of the strop. 3 indicates the condensed section of the strop. 4 indicates the face of the strop in a position in which it 70 can be treated with a view to produce the wavy surface referred to.

In practice the strop is made from a leather strap which may be of any good leather strop material. 75

The strap is first immersed in water until the surface is softened. With luke warm water an immersion of about 30 seconds more or less will be sufficient. Then the strap thus sufficiently moistened, is bent 80 around the form 5 and is drawn taut as indicated in Fig. 5. The force to draw the strap taut may be applied in any desired way or by any desired means, not shown. Then the operator will take a piece of pumice stone, not shown, and will rub the curved surface with light pressure until said surface becomes polished and very smooth. When the surface is thus rubbed until dry, it will seem, to the touch, to have 90 the smoothness of piano finish. The strap is thus treated throughout the entire stropping surface; and when the strap is straightened as in Fig. 2, and examined carefully, it will be found that the surface 95 is crinkled, so that to the touch of the finger tips, it affords a slight friction and upon careful examination it is found to have a wavy appearance.

In order to produce the above results it is 100 necessary to rub the leather with the pumice stone until the strap is dry.

The polish does not come upon the surface until the strap is dry. It is therefore understood that the length of time required to rub 105 down the surface to desired character will be greater with a well soaked strap than with a strap which has been only just im-

mersed. When the strap has been immersed in lukewarm water for some 30 seconds it is found to require rubbing and polishing for about one hour in a moderately dry atmosphere.

The time required for polishing also depends upon the speed of the polishing stone. The greater the speed the sooner drying and polishing of the surface is completed.

10 It is understood that the rubbing and polishing of the strap on the convex face stretches and condenses the surface so that when the strap has its fibers on the polished face, elongated, hardened and condensed, the 15 straightening of the strap throws the polished surface of the strap into a wavy, undulating and crinkly condition which greatly improves the operation of the strop.

The strop is used in practically the same

way as an ordinary razor strop, but the effect 20 is analogous to that of the use of a hone and after a hone edge is put on to the razor by use of the strop a finishing strop, not shown, will be employed to put the finished edge on the razor.

25 I claim.

1. A razor strop consisting of a leather strap having a polished condensed crinkled surface.

2. A razor strop comprising a strap of 30 leather having a flesh side, said flesh side being condensed, polished and wavy.

In testimony whereof, I have hereunto set my hand at Los Angeles, California, this 2nd day of April, 1920.

CHARLES E. GOODWIN.

Witness:

JAMES R. TOWNSEND.